

## UNITED STATES PATENT OFFICE

2,126,321

## PROCESS FOR FINISHING LEATHER ARTICLES

Hans Freudenberg and Philipp Haas, Weinheim, Germany, assignors to Freudenberg & Co. G. m. b. H., Frankfort-on-the-Main, Germany, a German company

No Drawing. Application November 1, 1934, Serial No. 751,113. In Germany August 28, 1933

10 Claims. (Cl. 12—142)

For the manufacture of leather goods, particularly high-grade footwear, leather which has been dressed in the leather factory is in general employed. This process of dressing consists in 5 several individual treatments, which commence after the drying of the leather, such as pressing, pommelling, polishing, pounding, ironing and the like, some of which are several times repeated.

In the manufacture of shoes, boots and other 10 articles from leather dressed in the leather factory, the leather more or less loses its good appearance—it becomes dull and soiled or stained. It is consequently necessary to impart a satisfactory appearance to the footwear by the application of so-called finishes. The finishing of 15 leather goods has in general been hitherto effected by first washing them, whereby the dressing produced in the leather factory is to a considerable extent again removed, and then applying the usual shoe-finishing preparations, which are, for example, prepared from shellac, 20 wax and the like materials.

This invention has as its object the manufacture from non-dressed or only partially dressed 25 leather of finished articles, particularly footwear, which satisfy the present high requirements, particularly with regard to colour, purity of colour, gloss or polish and the like.

According to this invention it has been found 30 that goods or articles manufactured from non-dressed or only partially dressed leather, particularly footwear, i. e. goods or articles which, owing to their appearance, especially with regard to colour and polish, are not customarily marketed, can be converted into high-grade goods, 35 which satisfy all trade requirements, by employing for the finishing of the non-dressed or only partially dressed leather articles, particularly footwear, solutions or preferably aqueous emulsions of polymers of acrylic compounds, which, 40 because of the size of the molecule or molecular framework, remain adhering substantially to the outer layer of the upper leather and consequently do not cause the grain side of the leather to 45 become sticky and harden and, after drying, form coatings, which adhere satisfactorily to the base, are fast to water, if desired exert a more or less water-repelling action and do not impair the natural permeability of the leather.

50 Particularly suitable compounds are the polymers of acrylic acid and its esters or the polymers of homologues of such compounds, which in the solid condition possess the desired properties, such as, tenacity, elasticity, extensibility 55 and the like. Rubber, for example in the form

of latex or certain derivatives, e. g., halogen derivatives, of rubber, may also be employed, if desired in cooperation with the foregoing. In many cases it has proved to be advantageous to apply to the leather articles several polymers of acrylic compounds as aforesaid in combination, for example in the form of mixed polymers or mixtures of polymers, or in succession.

The solutions or emulsions may also contain admixtures for improving their properties, for 10 example softeners such as tricresyl phosphate or castor oil, oils such as oil of turpentine, wetting agents such as alcohol, protective colloids such as rubber latex or tragacanth, gloss-imparting agents such as shellac and albumin, if desired 15 several of such admixtures. In many cases it has proved to be advantageous also to add drying oils.

According to an important embodiment of this invention pigment colours or soluble dyestuffs or 20 colours of both kinds are incorporated with the solutions or emulsions. In this way it is possible to impart any desired colour to the footwear, for example shoes, during the finishing process.

The polymers of acrylic compounds may be 25 dissolved in the usual organic solvents and be employed in the form of such solutions, which may, if desired, also contain certain admixtures. In the case of chlorinated rubber solutions an addition of castor oil has in many cases proved 30 to be advantageous.

It has however been found according to this invention that the use of expensive organic solvents can be entirely or to a large extent avoided and that the polymers of acrylic compounds can 35 be employed in the form of aqueous emulsions, which are free from organic solvents or may, if desired, also contain relatively small quantities of organic liquids. These aqueous emulsions may, for example, be prepared as follows:

Starting materials, which are capable of yielding 40 polymers of the desired properties, such as vinyl acetate, acrylic acid, acrylic acid methyl or ethyl esters, meta-acrylic acid esters and the like, or mixtures of the same are polymerized by 45 known methods, for example by heating in the presence of polymerization accelerators. The polymerization need not be carried to completion. The procedure may rather be adopted of carrying out the process of polymerization only 50 to the point of formation of more or less viscous intermediate products and employing the latter for the preparation of the aqueous emulsions. For the production of the aqueous emulsions mixtures of water and organic liquids may also 55

be employed. The polymer or mixture of polymers may, for example, be dissolved in organic solvents or be diluted with organic liquids and the resulting products be converted into aqueous emulsions. Admixtures of the aforesaid kind 5 may be incorporated with the emulsions during the process of their preparation or subsequent thereto.

It has proved to be advantageous to subject 10 the emulsions before their application to a natural or artificial ageing process, for example by allowing the emulsions to stand for a few hours or longer, if desired at raised temperature, for example at 40° to 50° C. In many cases it has 15 proved to be advantageous to add alkaline-reacting substances, particularly ammonia.

In carrying the process of this invention into effect the procedure may for example be followed 20 of working up the leather, which has been subjected to the usual treatments of removing acid, colouring, greasing, burnishing, drying and pressing in order to render the grain compact, into completely fabricated articles, for example, 25 shoes without the application of further treatments, particularly pounding, and imparting to the same the desired appearance with regard to polish, colour and the like, by applying finishes in accordance with the present invention.

In the manufacture of the leather a layer of 30 mucilage or the like may in this case be applied at any stage of the sequence of operations. On the other hand the repeated application of albumin or blood polishes hitherto customary may be dispensed with. The process of staining or 35 colouring may also be omitted in the manufacture of the leather and the staining or colouring be effected exclusively by the process of finishing according to this invention, alternatively articles may be manufactured from leather, 40 which has been only preliminarily coloured, and the final colour be imparted to these articles on finishing.

The application of the finishes according to 45 this invention is effected in a very simple manner, by applying the same, e. g., by brushing on, for example, to the shoe. By the successive application of several coats special effects may be obtained, for example with regard to polish and colour. The individual coats may contain different polymers of acrylic compounds; they may 50 contain different colouring matters or be in part uncoloured and in part contain colours. When employing colour-containing coats, colour-free finishes may be employed as covering coats. After 55 applying one coat, for example an aqueous emulsion, this is with advantage first allowed to dry for a few minutes, after which the next coat is applied and this again allowed to dry for a few minutes and so on.

The finishes according to this invention adhere 60 fast to the base and, after drying, impart to the article, for example footwear, treated therewith the desired colour and polish, without the leather base being unfavourably influenced, for example 65 by being rendered sticky or hard. The coatings are distinguished by being satisfactorily waterproof and frequently by possessing water-repelling effects. The latter can, if necessary, be further increased by suitable additions.

The invention enables high-grade leather articles, particularly footwear, which fulfil all requirements, particularly with regard to soft texture, fine grain, polish, colour and the like, to 70 be manufactured from non-dressed or only partially dressed, non-coloured or only preliminarily

coloured leather. Footwear of any desired colour, shade and polish can be manufactured. Special effects can be produced by applying several colours in succession. It is also possible to colour certain parts of one and the same article of 5 footwear with one colour, and other parts with other colours and in this way to obtain combined effects. The invention also possesses inter alia the great advantage that footwear manufactured from non-coloured or only partially 10 coloured (preliminarily coloured) leather can be kept in reserve and be subsequently coloured directly before being sold in accordance with the prevailing fashion.

It is already known to prepare solutions or 15 emulsions of compounds of high molecular weight of the kind hereinbefore described and to employ them for the most varied purposes, including the treatment of leather. The use of the hereinbefore described solutions and particularly 20 emulsions as finishes for leather articles, particularly footwear, which have been manufactured from non-dressed or only partially dressed leather is, however, new. It is not possible to produce the effects of the present invention with the known shoe finishes, manufactured from shellac, wax and the like. The hereinbefore described applicability of the solutions and emulsions as finishing agents and the particular 25 advantages accruing from the application of 30 these agents could not have been concluded from the applicability of solutions of polymers of unsaturated compounds and the like substances as agents for the treatment of leather, for example in tanneries. It could in no way have been foreseen that it would be possible, under the application 35 of the finishing agents hereinbefore described, to manufacture leather articles, such as shoes, boots and the like from non-dressed or only partially dressed leather, and to impart to 40 the same the desired polish and colour, without any injury to the leather taking place or other disadvantages appearing.

#### Examples

1. 100 parts of a commercial aqueous emulsion of a polymer of acrylic acid derivatives are treated with 5 parts of concentrated aqueous ammonia, allowed to stand for 3 days, at 50° C. and then mixed with 40 to 100 parts of a black 50 pigment, such as is usually used for dressing black leather.

Shoes manufactured from non-dressed leather, which have not been subjected to the usual final dressing treatment, are treated with the 55 aforesaid finish by brushing the latter on and allowing to dry. This treatment is repeated three times and, if desired, a final coat of an emulsion of the acrylic acid derivative polymer, which contains no colouring matter, is applied. 60 The treated shoes have a black colour of excellent appearance. The grain surface of the leather is soft and elastic.

In order to impart a lacquer-like polish to the toe cap, this is two or three times brushed over 65 with an emulsion of a polyvinyl compound, containing no colouring matter, or a colour-free or colour-containing solution of chlorinated rubber, which may, if desired, contain an addition of castor oil.

2. Shoes made of non-dressed or only partially dressed leather are, if necessary, washed and treated with a finish prepared as follows:

100 parts of a 25% aqueous emulsion of polymers of acrylic acid esters are mixed with 100 parts 75

of a colouring solution, containing 1 to 2% of a black aniline dye and the same quantity of lamp-black pigment, a small quantity of 1% ammonia, 0.5% of shellac, 0.3% of Turkey red oil and, if desired, small quantities of xylene or other organic solvents in addition and preferably subjected, before mixing with the polymer solution, to a boiling down treatment of several hours duration.

10 The shoes are brushed over two or three times with this finish, each coat being allowed to dry before the application of the next coat.

15 3. A trunk made of raw leather is brushed over with a coat of a usual brown pigment colour mixture, with the addition of aniline colours and an aqueous emulsion of polymers of acrylic acid- and polyvinyl compounds. The edges are then colored in darker tones than the surfaces with a suitably coloured emulsion.

20 4. The term "partly dressed leather" as used in the specification and claims is intended to cover leather which has been subjected to the following usual treatments: removing acid, greasing, drying and pressing, and, if desired, coloring, applying a layer of mucilage and burnishing, but which has not been subjected to pounding and to repeated applications of albumin or blood polishes.

What we claim is:

30 1. A process for the manufacture of finished leather articles which consists in assembling the articles from parts of partly dressed leather and finishing the assembled articles by applying thereto a coating of liquids containing polymers of acrylic compounds which possess the property of drying on with the formation of adhering layers, which are fast to water, tenacious, elastic and extensible and do not harden the grain side of the leather.

2. A process for the manufacture of finished footwear which consists in assembling the footwear from parts of partly dressed leather and finishing the assembled articles by applying thereto a coating of liquids containing polymers of acrylic compounds which possess the property of drying on with the formation of adhering layers, which are fast to water, tenacious, elastic and extensible and do not harden the grain side of the leather.

10 3. A process according to claim 1, in which said liquids also contain colours, such as pigment colours and organic colours.

4. A process according to claim 1, in which said liquids comprise aqueous emulsions which 15 contain alkaline substances.

5. A process according to claim 1, in which the leather is uncoloured, said liquids also containing colours.

6. A process according to claim 1, in which 20 the leather is preliminarily coloured, said liquids also containing colours.

7. A process according to claim 1, in which the finishes are applied in several coats, the individual coats containing different polymers of 25 acrylic compounds.

8. A process according to claim 1, in which the finishes are applied in several coats, the individual coats containing different colours.

9. A process according to claim 1, in which 30 the finishes are applied in several coats, some of said coats being colourless and others containing colours.

10. A process according to claim 1, in which the finishes are applied in several coats, said 35 liquids comprising in part aqueous emulsions, and in part solutions.

HANS FREUDENBERG.  
PHILIPP HAAS.